

Nov. 4, 1941.

C. WENTWORTH

2,261,425

METHOD OF MAKING PARAMAGNETIC MATERIALS

Filed Jan. 31, 1940



Inventor  
*Chandler Wentworth*

By

Attorney

Patented Nov. 4, 1941

2,261,425

# UNITED STATES PATENT OFFICE

2,261,425

## METHOD OF MAKING PARAMAGNETIC MATERIALS

Chandler Wentworth, Haddon Heights, N. J., assignor to Radio Corporation of America, a corporation of Delaware

Application January 31, 1940, Serial No. 316,692

2 Claims. (Cl. 148—1)

This invention relates to the manufacture of cores and other structures formed of comminuted paramagnetic materials.

The prior art recognizes that structures formed of curved or spherical magnetic or paramagnetic particles exhibit a higher resistance to eddy current losses than similar structures formed of irregular or angular particles of the same material. This is so because such curved or spherical particles can be insulated and compressed into a coherent structure with a minimum of damage to the insulation which must necessarily be present between the individual particles in the finished structure.

While various methods are known for producing such nonangular particles, the usual methods suffer the common disadvantage that their practice results in the production of particles which are coated with an oxide of the metal or alloy of which the particles are formed. It is of course true that such oxide coatings may be utilized as the insulating material which serves to electrically isolate the individual particles in the finished structure; however, the very presence of such oxides results in a structure of lower permeability than would be the case if certain other more efficient insulating material were to be employed.

Accordingly, the principal object of the present invention is to provide an improved method of producing unoxidized spherical or curved paramagnetic particles.

Other objects and advantages will be apparent and the invention itself will be best understood by reference to the following specification and to the accompanying sectional view of an apparatus which may be employed in the practice of the method of the invention.

In carrying the invention into effect, it is preferable to start with a batch 1 of oxidized or partially oxidized powdered iron, nickel, magnetite ore, or alloys of nickel and iron, and to separate

the powdered particles as by gently agitating a sieve 2 or the like in which the batch is contained. The separate particles are rendered molten by contact with a hot gaseous medium emanating from a flaming liquid fuel 3 such, for example, as alcohol, contained in a tank or receptacle 4. It may be that the particles, upon having the sieve, enter a gaseous strata or zone A wherein they are subject to some degree of oxidation. If this is indeed the case, the oxide or oxides are effectively reduced upon the conversion of the particles to the molten state, say in the second zone B. It is while in the molten state that the particles assume a curved or substantially spherical contour which is preserved upon their partial solidification during their passage through the lower temperatures prevailing in the nonoxidizing gaseous zone C immediately above the alcohol or other non-aqueous liquid 3 in which they are collected and cooled.

After the now cool rounded or spherical metallic particles are removed from the nonoxidizing medium in which they are collected, they may be coated with an insulating substance of a type calculated to ensure high permeability. Among the recommended insulating coating materials are iron and zinc salts, which may be formed by treating the particles with phosphoric acid containing some (say 12% by weight) zinc.

What is claimed is:

1. Method of making paramagnetic particles of substantially curved contour which comprises dropping separate molten particles of a magnetic material into flaming alcohol.
2. Method of making unoxidized paramagnetic particles of substantially curved contour which comprises subjecting separate comminuted particles of a magnetic material to an alcohol flame to render said particles molten and then solidifying said particles in fluid alcohol.

CHANDLER WENTWORTH.